

1,410,499.

A. PACZ.  
METAL AND ITS MANUFACTURE.  
APPLICATION FILED FEB. 20, 1917.

Patented Mar. 21, 1922.



INVENTOR  
ALADAR PACZ

BY *Alfred S. Davis*  
HIS ATTORNEY

# UNITED STATES PATENT OFFICE.

ALADAR PACZ, OF CLEVELAND, OHIO, ASSIGNOR TO GENERAL ELECTRIC COMPANY, A CORPORATION OF NEW YORK.

## METAL AND ITS MANUFACTURE.

1,410,499.

Specification of Letters Patent. Patented Mar. 21, 1922.

Application filed February 20, 1917. Serial No. 149,915.

To all whom it may concern:

Be it known that I, ALADAR PACZ, a citizen of the United States, residing at Cleveland, in the county of Cuyahoga, State of Ohio, 5 have invented certain new and useful Improvements in Metals and Their Manufacture, of which the following is a specification.

The object of my invention is to produce 10 tungsten metal which will retain to a much higher degree than heretofore its original properties after being subjected to high temperatures. In the case of incandescent lamp filaments, the high temperatures at which 15 they are run have caused them to elongate and sag between their supports. This is especially noticeable in coiled filaments, and in gas filled lamps this tends to reduce the efficiency of the lamp on account of the increased cooling effect on the filament. By 20 means of my invention the sagging is substantially eliminated and "offsetting" of the filament is substantially prevented, during a normal or commercially useful life of the 25 lamp.

In the preferred form of my invention I bring into intimate association with tungsten a material which will have the desired influence upon the grain growth of the metal. 30 I precipitate, simultaneously, compounds from which the metal is to be directly reduced with the material or compound which is to accomplish the desired result. The material after precipitation will remain in intimate association with the metal even after the same has been reduced by the ordinary means, i. e., reducing gases. During the subsequent formation of the metal into ingots or bars, the material should be such 35 that it will be removed as by volatilization. A material should be used which will have a fairly high volatilization point which is preferably somewhat lower than the sintering point of the metal.

40 Considering my invention from the physical standpoint, the presence of the material has an influence on the grain growth of the metal. When the metal reaches the temperature at which extensive grain growth 45 would ordinarily take place, the presence of this material intimately associated with the tungsten particles has a marked effect on the shape and size of the tungsten grains. The ingot of tungsten thus produced, 50 whether it be due to the fact that the grains

have not reached the equilibrium grain size or to other causes, is particularly susceptible to grain growth during subsequent heat treatments.

The probable reason why filaments made 60 according to my invention do not sag, is that the structure is comparatively coarse grained. The coarse grained filament produced by means of my invention does not "offset" so as to cut short the life of the lamp appre- 65 ciably.

As hereinbefore stated, the material which is intimately incorporated with the metal should be such that it will be volatilized out after the metal has reached the temperature 70 of rapid grain growth. Tungsten above 1500° C. shows rapid grain growth, and I may use silica, or compounds containing it, as the material, incorporated very intimately as heretofore explained. By the time the 75 tungsten has reached the sintering temperature the silica and the compounds containing it are volatilized out.

In order to comply fully with the requirements of the patent statutes, I will now describe one method or process embodying my invention and also modifications thereof. However, it is to be understood that the scope of my invention is such that many changes and substitutions will readily suggest themselves to those skilled in the art, and, as indicated, in the appended claims, are to be considered as forming part thereof.

A fusion of materials is first made which is quite similar to that disclosed in my Patent Number 1,299,017 issued April 1, 1919. 80 1400 grams of commercial tungstic acid, 620 grams commercial sodium carbonate, 620 grams commercial potassium carbonate, and 300 grams commercial sodium nitrate are 85 mixed with water to a paste. I have found that half or more of the potassium carbonate may be replaced by sodium carbonate without affecting the results, the object being to obtain a good fusion. This paste is dried 90 on a hot plate and fused with a torch for about fifteen minutes, after which the fusion is dissolved in water, filtered and diluted to about six liters. This we will term solution A.

100 A mixture is then made of 180 grams commercial silicic acid, 620 grams commercial  $K_2CO_3$  and 150 grams commercial  $NaNO_3$  with water to a paste which is dried and 105 fused. The object is to produce a silicate 110

which will be readily incorporated with the tungstic acid in the subsequent portion of the process. An alkaline silicate such as produced by the specific example given is readily soluble and efficacious for this purpose. The fusion is dissolved in water, filtered and diluted to 5 liters. This may be termed solution B.

About 250 cubic centimeters of solution 10 B are added to 3 liters of solution A. The whole solution is then boiled with steam and poured into a boiling solution containing about 1500 cubic centimeters of HCl and 1500 cubic centimeters of H<sub>2</sub>O, preferably 15 through a funnel. The precipitate is allowed to settle, the liquid decanted, and the precipitate separated by filtration. The precipitate is then washed with hot H<sub>2</sub>O until the filtrate becomes milky. The precipitate 20 is then dried and ignited in a quartz dish. It is reduced in hydrogen in boats, each boat containing about 100 grams. The metal thus produced may be termed metal A.

The metal A may be pressed up and sintered to produce tungsten slugs which may be drawn into filaments having the non-sag and other characteristics hereinbefore described. I prefer, however, in order to obtain greater uniformity of product to continue the operation as follows:

About 1200 grams of metal A are mixed with about 1200 grams of the oxide from which metal A was reduced, the mixture being very intimate and being performed preferably in 5 a tumbling mill. The mixture is then reduced as before although 150 gram charges may be here used. The metal thus produced may be termed metal B. It is then sieved, pressed into ingots and sintered in the usual 0 way as set forth in the Coolidge Patent No. 1,082,933.

As a modification of the above described process, solution B may be added directly to the fusion from which solution A is made. 5 This is preferably done by utilizing the proper proportion as heretofore stated of solution B in making the paste which is dried and fused and dissolved to form solution A.

The metal obtained from the first method above described I have called "218", a purely arbitrary name. I have produced a metal differing in appearance and physical characteristics from "218" metal by adding a solution of boric acid to chemically pure WO<sub>3</sub>, evaporating, drying, igniting and reducing. The metal thus produced when made into wire is not superior to "218" in non-sagging or non-offsetting characteristics, but a combination of this method with that for producing "218" in which the WO<sub>3</sub> from the latter is mixed with that from the former produces a metal which I term "Z" and which is efficacious in the production of non-sagging and non-offsetting filaments. To

produce this metal one method which I have practiced is to mix 1 kilogram of the tungstic oxide from which metal A is reduced in the "218" process with a solution of 12.5 grams fused B<sub>2</sub>O<sub>3</sub> in 500 cubic centimeters of water. This mixture is evaporated, dried, ignited and reduced. The resulting metal is blacker than "218", flows more readily and possesses at least one-third larger volume than "218" although reduced under exactly the same conditions.

The tungsten ingots produced according to my invention usually have fine grains, as for example, between 2500 and 6500 grains per square millimeter. In the case of the "218" ingots analyses have shown that the percentage of non-metallic material is below two-tenths of one per cent and in many cases below one-tenth and even one-twentieth of one per cent.

When the tungsten metal produced by any of the methods above described is to be made into a filamentary body, the method described in the Coolidge Patent No. 1,082,933 for drawing or otherwise working down the ingots is practiced. Where the wire is to be used at high temperatures such as in incandescent electric lamps it should be given a preliminary heat treatment or aging. This helps to secure the non-sag characteristics of the wire made according to my invention. One procedure followed with good results with the ordinary 110-115 volts lamps was to run at 30 volts for 2 minutes and then at steps of 5 volts each for two minutes up to 60 volts. After this the wire was run at 115% voltage for 15 minutes.

In the accompanying drawing I have shown, in elevation, lamps, the filaments of which are made according to my invention. Figs. 1, 2 and 3 are front elevations of these lamps, while Figs. 4 and 5 are partial side elevations showing the filaments and supports. All of these lamps may be of ordinary voltage, i. e. 110 volts, and of any of the ordinarily used wattages. The lamps shown in Fig. 1 and Fig. 2 are of the gas-filled type disclosed in the Langmuir Patent No. 1,180,159, and have coiled filaments 11 and 12. The lamp shown in Fig. 3 is a vacuum lamp having the coiled filament 13. The support 14 is provided for the single loop filament 11 and the support 15 for the single loop filament 13. Heretofore it was impractical to make a lamp like this, having a single coiled loop filament for use at ordinary voltages. The non-sag characteristics of my wire render this construction possible for all of the ordinary voltages and wattages.

The tests on 50 and 100 watt lamps embodying the construction shown in Figs. 1 and 2 of the drawing show that substantially all of the sagging occurs during the aging of the lamp. This is when the lamp filament is

given the heat treatment hereinbefore referred to. The sagging was greater in the case of the construction shown in Fig. 1 than in that shown in Fig. 2 on account of the fact that in the latter there are more supports. In the construction shown in Fig. 1 in the case of 50 watt 115 volt lamps in which the filament was 1.62 mils in diameter and which was made by coiling on a mandrel of 5 mils diameter, the turns per inch originally ran from 421 to 430 and after aging the average decrease in the number of turns per inch was from 18 to 24. This was under 5%. In the case of the construction shown in Fig. 2 the decrease was from 1 to 6 turns, or under 2%. In the case of 100 watt 115 volt lamps, in which the filament diameter was 2.63 mils and the filament was shaped by coiling upon an 8 mil mandrel the number of turns per inch originally ran from 257 to 269. After aging, in the case of the construction shown in Fig. 1 the decrease in number of turns was from 0 to 10 or less than 5% and in the case of construction shown in Fig. 2 it was from 0 to 6 turns per inch, or less than 3%. In one case, after total life of a 100 watt lamp, the number of turns decrease in the case of the construction shown in Fig. 1 was 12, while in the construction shown in Fig. 2 it was 4.

What I claim is:

1. The process of producing substantially non-sagging and non-offsetting tungsten filaments, which includes intimately associating finely divided tungsten and a material which volatilizes mainly at temperatures within the range of rapid grain growth of the tungsten and thereafter sintering the tungsten into a coherent body.
2. The process of producing substantially non-sagging and non-offsetting tungsten filaments, which includes intimately associating finely divided tungsten and a material which volatilizes mainly at temperatures within the range of rapid grain growth of the tungsten, thereafter sintering the tungsten into an ingot, and working such ingot into filament form.
3. The process of producing substantially non-sagging and non-offsetting tungsten filaments, which consists in reducing a tungsten oxide intimately associated with a material which volatilizes mainly at temperatures within the range of rapid grain growth of the tungsten and thereafter producing a coherent body by sintering a compacted body of the product of such reduction.
4. The method of producing substantially non-sagging and non-offsetting tungsten filaments, which includes producing a coherent body of tungsten by sintering finely divided tungsten having intimately associated therewith a compound or compounds containing silicon and oxygen and volatilizing mainly at temperatures within the range of rapid grain growth of the tungsten, and

at temperatures within the range of rapid grain growth of the tungsten.

5. The method of producing substantially non-sagging and non-offsetting tungsten filaments, which includes producing a coherent body of tungsten by sintering finely divided tungsten having intimately associated therewith a compound or compounds containing silicon, oxygen and an alkali metal, and volatilizing mainly at temperatures within the range of rapid grain growth of the tungsten.

6. The method of producing substantially non-sagging and non-offsetting tungsten filaments, which includes producing a coherent body of tungsten by sintering finely divided tungsten having intimately associated therewith a compound or compounds, containing silicon, oxygen and potassium, and volatilizing mainly at temperatures within the range of rapid grain growth of the tungsten.

7. The method of producing tungsten filaments, which includes producing an ingot by heating finely divided tungsten having intimately associated therewith a compound or compounds, containing silicon and oxygen, and volatilizing mainly at temperatures within the range of rapid grain growth of the tungsten, and thereafter working said ingot down to filament form.

8. The method of producing tungsten filaments, which includes producing an ingot by sintering finely divided tungsten having intimately associated therewith a compound or compounds, containing silicon, oxygen and an alkali metal, and volatilizing mainly at temperatures within the range of rapid grain growth of the tungsten and thereafter working said ingot down to filament form.

9. The method of producing tungsten filaments, which includes producing an ingot by sintering finely divided tungsten having intimately associated therewith a compound or compounds containing silicon, oxygen and potassium, and volatilizing mainly at temperatures within the range of rapid grain growth of the tungsten, and thereafter working said ingot down to filament form.

10. The method of producing tungsten filaments, which includes reducing a tungsten oxide intimately associated with a compound or compounds containing silicon and oxygen, and volatilizing mainly at temperatures within the range of rapid grain growth of the tungsten, and thereafter producing a coherent body by sintering a compacted body of the product of such reduction.

11. The method of producing tungsten filaments, which includes reducing a tungsten oxide intimately associated with a compound or compounds containing silicon, oxygen and an alkali metal, and volatilizing mainly at temperatures within the range of rapid grain growth of the tungsten, and

thereafter producing a coherent body by sintering a compacted body of the product of such reduction.

12. The method of producing tungsten filaments, which includes reducing a tungsten oxide intimately associated with a compound or compounds containing silicon, oxygen and potassium, and volatilizing mainly at temperatures within the range of 10 rapid grain growth of the tungsten and thereafter producing a coherent body by sintering a compacted body of the product of such reduction.

13. The method of producing tungsten filaments, which consists in reducing a tungsten oxide intimately associated with a compound or compounds containing silicon and oxygen and volatilizing mainly at temperatures within the range of rapid grain growth of the tungsten, producing an ingot by sintering a compacted body of the product of such reduction and working down the said ingot.

14. The method of producing tungsten filaments, which consists in reducing a tungsten oxide intimately associated with a compound or compounds containing silicon, oxygen and an alkali metal and volatilizing mainly at temperatures within the range of 30 rapid grain growth of the tungsten and producing an ingot by sintering a compacted body of the product of such reduction and working down the said ingot.

15. The method of producing tungsten filaments, which consists in reducing a tungsten oxide intimately associated with a compound or compounds containing silicon, oxygen and potassium and volatilizing at temperatures within the range of rapid grain growth of the tungsten and producing an ingot by sintering a compacted body of the product of such reduction and working down the said ingot.

16. The process of producing substantially non-sagging and non-offsetting tungsten filaments, which includes intimately associating tungsten oxide and a material which volatilizes mainly at a temperature within the range of rapid grain growth of tungsten, reducing a portion of said oxide to metal, mixing said metal with another portion of said oxide, reducing said mixture, and working the product of said reduction into filamentary form.

17. The process of producing substantially non-sagging and non-offsetting tungsten filaments, which includes preparing tungsten oxide intimately associated with an alkali metal and an oxide of silicon, reducing said tungsten oxide to metal, mixing said metal with another portion of said oxide, reducing said mixture, and working the product of said reduction into filamentary form.

18. The process of producing substantially non-sagging and non-offsetting tungsten filaments, which includes preparing tungsten oxide intimately associated with potassium and an oxide of silicon, reducing a portion of said oxide to metal, making a 7 mixture of said metal and another portion of said oxide, reducing said mixture, and working the product of said reduction into filamentary form.

19. The process of producing substantially non-sagging and non-offsetting filaments, which includes precipitating a tungsten compound from a solution containing as constituents an alkali metal and a silicon oxide and reducing the precipitate substantially to tungsten metal.

20. The process of producing substantially non-sagging and non-offsetting filaments, which includes precipitating a tungsten compound from a solution containing 85 as constituents an alkali metal and a silicon oxide, reducing the precipitate substantially to tungsten metal, forming an ingot therefrom and working the same into filament form.

21. The process of producing substantially non-sagging and non-offsetting filaments, which includes precipitating a tungsten compound from a solution containing as constituents potassium and a silicon oxide 95 and reducing the precipitate substantially to tungsten metal.

22. The process of producing substantially non-sagging and non-offsetting filaments, which includes precipitating a tungsten compound from a solution containing 100 as constituents potassium and a silicon oxide, reducing the precipitate substantially to tungsten, forming an ingot therefrom and working the same into filament 105 form.

23. A tungsten filament containing materially less than three-fourths of one per cent of non-metallic material and substantially free from sagging and offsetting during a normal or commercially useful life.

24. A coiled tungsten filament containing materially less than three-fourths of one per cent of non-metallic material and substantially free from sagging and offsetting 115 during a normal or commercially useful life.

25. A filament for electric incandescent lamps or other devices, composed substantially of tungsten and made up mainly of a number of comparatively large grains of 120 such size and contour as to prevent substantial sagging and offsetting during a normal or commercially useful life for such a lamp or other device.

26. A drawn filament for electric incandescent lamps or other devices, composed substantially of tungsten and made up 125 mainly of a number of comparatively large

grains of such size and contour as to prevent substantial sagging and off-setting during a normal or commercially useful life for such a lamp or other device.

5 27. A filament for electric incandescent lamps or other devices, composed of tungsten containing less than three-fourths of one percent of non-metallic material and made up mainly of comparatively large 10 grains of such size and contour as to prevent substantial sagging or offsetting during a normal or commercially useful life for such a lamp or other device.

28. A coiled filament composed substantially of tungsten and capable of use in an electric incandescent lamp without either substantial sagging or offsetting during a normal or commercially useful life.

15 29. A coiled filament composed mainly of drawn tungsten and capable of use in an electric incandescent lamp without substantial sagging and without substantial offset-

ting during a normal or commercially useful life.

30. A drawn filament composed mainly of tungsten and capable of use in an electric incandescent lamp without substantial sagging and without substantial offsetting during a normal or commercially useful life.

31. A filamentary body composed substantially of tungsten and adapted to be mounted in an incandescent electric lamp and after it has been aged, capable of a normal or commercially useful life without substantial sagging and without substantial offsetting.

32. A drawn tungsten wire adapted for use as an incandescent lamp filament and capable after aging, of a normal or commercially useful life without substantial sagging and without substantial offsetting.

In witness whereof, I have hereunto set my hand this 16th day of February, 1917.

ALADAR PACZ.

### DISCLAIMER

1,410,499.—Aladar Pacz, Cleveland, Ohio. METAL AND ITS MANUFACTURE. Patent dated March 21, 1922. Disclaimer filed November 10, 1933, by the assignee, *General Electric Company*.

Therefore enters this disclaimer to so much of the statement on lines 52 to 59 of page 2 of the printed patent specification as might imply or tend to imply that by "adding a solution of boric acid to chemically pure  $WO_3$ , evaporating, drying, igniting and reducing" alone, it is possible to produce commercially useful non-sagging and non-offsetting tungsten filaments.

[*Official Gazette December 5, 1933.*]

### DISCLAIMER

1,410,499.—Aladar Pacz, Cleveland, Ohio. METAL AND ITS MANUFACTURE. Patent dated March 21, 1922. Disclaimer filed June 16, 1938, by the assignee, *General Electric Company*.

Hereby enters this disclaimer of claims 23, 24, 28, 29, 30, 31, and 32 of said patent.

And further disclaims from the scope of each of claims 25, 26, and 27 all filaments except filaments of the character therein described, which are made up mainly of grains of a size and contour comparable to the grains of filaments produced in accordance with the processes described in the specification at page 1, line 89 to page 2, line 49, and page 2, lines 89 to 102.

[*Official Gazette July 12, 1938.*]